

## UNITED STATES PATENT OFFICE

2,580,038

MINERAL OIL CONTAINING RESINIFIED  
ESTERS OF SALICYLIC ACIDLouis A. Mikeska, Westfield, N. J., assignor to  
Standard Oil Development Company, a corpo-  
ration of DelawareNo Drawing. Application September 30, 1949,  
Serial No. 119,019

2 Claims. (Cl. 252—57)

1

This invention relates to new and useful condensation products having pour point depressing characteristics and to a lubricating composition containing such material. The invention particularly relates to a pour point depressant formed by condensing an ester of salicylic acid in which the alcohol contributed portion of the ester contains from 8 to 24 carbon atoms with a resinifying agent exemplified by an aldehyde.

The use of salicylic acid as an intermediate compound for the formation of lubricating oil additives is known in the art. For example, Reiff in U. S. Patent 2,147,545, discloses that his lubricating oil additives, which comprise condensation products of chlorinated ester waxes and phenols, may be acylated by using the chloride or anhydride of a carboxylic acid or the acid itself and discloses along with a series of others, salicylic acid. Again in U. S. Patent 2,339,692, Finley teaches that a lubricating oil containing the calcium salt of the capryl ester of salicylic acid results in a good lubricating oil composition. In U. S. Patent 2,348,461, Finley et al. discloses that the thermal stability of a motor oil is increased by the addition of a mixed calcium salt of an alkyl phenol sulfide and an alkyl ester of salicylic acid. U. S. Patent 2,373,286, teaches a reaction product of a phosphorus pentahalide with salicylic acid improves a lubricating oil blend by reducing corrosion. U. S. Patent 2,458,527, teaches the use of an aldehyde-poly-amine-hydroxy aromatic carboxylic acid condensation product as an all purpose additive, especially as a pour depressant.

It has now been found and forms the subject of this invention that a long chain ester of salicylic acid may be condensed with a resinifying agent such as formaldehyde, or a formaldehyde derivative, to yield a condensation product which has exceptional qualities as a pour depressing additive.

The ester of salicylic acid is formed by reacting with the acid a straight chain alcohol or a mixture of alcohols containing from 8 to 24 carbon atoms per molecule. Although any of the alcohols included above are operable it is preferred to use alcohols having a carbon chain length of from 10 to 16, lauryl alcohol being especially preferred.

The esters of salicylic acid obtained by the esterification of the acid are then condensed with a resinifying agent. Operable among the common resinifying agents are, in general, the aldehydes, and, in particular, formaldehyde or its

5 derivatives such as paraformaldehyde, trioxane, hexamethylenetetramine and the like. In the condensation reaction exemplifying this invention and its preferred embodiment, a mixture of chloromethyl ethyl ether and stannic chloride is used to form the formaldehyde in situ.

To describe the condensation reaction generally the ingredients in equimolar proportions are mixed and heated with stirring at a temperature 10 from about 100°-200° C. The reaction is continued for a time varying between 4-10 hours. The preferred temperature is from 100°-150° C., and the time preferred is from about 2 to about 7 hours. It is to be understood of course that the 15 temperatures and times used will depend upon the molecular weight of the product it is desired to obtain. The molecular weight will vary proportionally with the time and temperature of the reaction, and with the relative amounts of the 20 reactants used.

If it is desired the salicylic acid esters may first be condensed with sulfur monochloride or sulfur dichloride, which condensation may then be followed by the resinifying reaction with the formaldehyde. The condensates in this case are effective not only as pour point depressants but also as anti-oxidants. Metal salts of the condensate such as the barium, calcium, manganese, strontium, aluminum, magnesium, salts, etc., are also 25 effective as lube oil detergent additives.

The invention will be more clearly explained by a consideration of the following example.

## EXAMPLE

35 A three-way flask equipped with a thermometer and a return condenser was charged with 61.2 grams (0.2 mols) of lauryl salicylate and 18.9 grams (0.2 mols) of chloromethyl ethyl ether. To this was then added 5 grams of stannic chloride, whereupon the mixture was heated with 40 stirring at 85° C. for one and one half hours. At this point a water trap was inserted between the condenser and the reactor and the temperature was gradually raised to 110° C. 8 cc. of a distillate, which collected in the water trap, was 45 removed.

A qualitative test at this point seemed to indicate that the condensation had not gone far enough. Hence, another 18.9 grams of chloromethyl ethyl ether were added and the mixture 50 was refluxed for 5 additional hours. The temperature gradually rose from 90° to 130° C. The reaction mixture thickened considerably during this heating.

The product was then poured into water, acidified

fied with hydrochloric acid, and extracted with ether. The extract was washed and dried over sodium sulfate. On removal of the solvent at 125° C. the condensate was obtained as a soft brown resinous material.

This condensate was evaluated as a pour point depressant in two oils, oil A, consisting of a paraffinic oil of SAE 10 grade and oil B consisting of a paraffinic oil of SAE 30 grade. Evaluation data of the pour point depressing tests according to regular A. S. T. M. procedure are given in the table below.

TABLE  
A. S. T. M. pour point test data

| Per cent by weight of additive | A. S. T. M. Pour Point |                    |
|--------------------------------|------------------------|--------------------|
|                                | Oil A <sup>1</sup>     | Oil B <sup>2</sup> |
| 0.....                         | +30° F.                | +20° F.            |
| 0.25.....                      | -15                    | (not run.)         |
| 0.50.....                      | -20                    | -15° F.            |
| 1.00.....                      | -35                    | (not run.)         |

<sup>1</sup> Oil A = A conventionally refined Mid-Continent Neutral of SAE 10 grade having a viscosity at 210° F. of 43.9 S. U. S. and a viscosity index of 101.

<sup>2</sup> Oil B = A conventionally refined Mid-Continent Neutral of SAE 30 grade having a viscosity at 210° F. of 63.7 S. U. S. and a viscosity index of 86.

(In pour stability tests 1/4% blend in A oil, the blend remained fluid at -20° F., which means that it had excellent pour stability.)

An examination of the data in the table above shows that the product of this invention was effective as a pour depressant in both low and high viscosity oils. The addition of the condensate lowered the pour point of the low viscosity oil from +30° F. to -35° F. in a 1% concentration and the high viscosity oil from +20° F. to -15° F. in a 1/2% concentration.

Although the pour point characteristics of the condensate of this invention are demonstrated herein by its addition to a mineral base lubricating oil, it is to be understood that this additive is completely compatible with other types of lubricating oils whether a naturally occurring mineral base type or a synthetic type oil.

The material of this invention may be used in

conjunction with other lubricating oil additives such as corrosion inhibitors, anti-oxidants, detergent additives, other pour depressants, and viscosity index improvers.

5 What is claimed is:

1. A lubricating oil composition consisting essentially of a major proportion of a mineral lubricating oil base stock having combined therein a minor proportion of a product formed by subjecting the compound having the general formula:



wherein R is a primary straight chained aliphatic hydrocarbon radical containing from 8 to 24 carbon atoms, to a temperature within a range of from about 50° to about 250° C. for a period of time within a range of from about 2 to about 20 hours in the presence of an equimolar proportion of formaldehyde.

2. A lubricating oil composition consisting essentially of a major proportion of a mineral lubricating oil base stock having combined therein from 0.2 to 5.0 per cent by weight of a compound formed by subjecting equimolar proportions of lauryl salicylate and chloromethyl ethyl ether to a temperature within a range of from about 100° to about 200° C. for a period of time within a range of from about 5 to about 15 hours in the presence of stannic chloride.

LOUIS A. MIKESKA.

#### REFERENCES CITED

The following references are of record in the file of this patent:

#### UNITED STATES PATENTS

| Number    | Name         | Date           |
|-----------|--------------|----------------|
| 2,256,442 | Reiff        | Sept. 16, 1941 |
| 2,269,186 | D'Alelio     | Jan. 6, 1942   |
| 2,357,359 | Reiff et al. | Sept. 5, 1944  |
| 2,380,305 | Gleason      | July 10, 1945  |
| 2,499,365 | De Groote    | Mar. 7, 1950   |